

# UNITED STATES PATENT OFFICE.

ROY A. ALEXANDER, OF BELLINGHAM, WASHINGTON.

## VARNISHED-SURFACE BURNISHER.

1,350,537.

Specification of Letters Patent. Patented Aug. 24, 1920.

No Drawing.

Application filed November 24, 1919. Serial No. 340,236.

To all whom it may concern:

Be it known that I, ROY A. ALEXANDER, a citizen of the United States, residing at Bellingham, in the county of Whatcom and State of Washington, have invented a new and useful Varnished-Surface Burnisher, of which the following is a specification.

The object of my invention is the production of a gum-solvent liquid suited for rubbing on varnished or finished surfaces to partly dissolve said varnish or finish and permit the forming, by rubbing, of a new surface of greater smoothness, density and hardness than the original, and better adapted for polishing with the aid of a suitable polishing liquid to be applied subsequently.

My composition consists of a mixture of a mineral oil, gum-solvent spirits, an acid, an alkali, a metal-cleaning substance, soap and water.

In preparing the composition I prefer to use the ingredients about as follows: 4 oz. paraffin oil,  $1\frac{1}{2}$  oz. turpentine, 3 oz. alcohol,  $\frac{1}{8}$  oz. acetic acid,  $\frac{1}{2}$  oz. ammonia,  $1\frac{1}{2}$  oz. Putz pomade, 1 oz. ivory soap, and 2 oz. water.

The several ingredients are thoroughly mixed by violent stirring and agitation.

To burnish a varnished or finished surface that is rough, bruised or scratched a small quantity of my burnisher is put on a piece of cheese cloth and applied to the surface by rapid rubbing movements. The applied liquid dissolves the surface, mixes with the dissolved material to form a quickly drying compound which rubs down to a hard, smooth surface well adapted for a foundation for the application of a suitable polishing liquid with which the surface can be subsequently finished with a high and durable gloss of great density and smoothness.

The Putz pomade used in my compound is an abrasive imported by J. A. Zibell of New York, N. Y., and comprises a mixture of finely ground rotten stone and pumice stone with vaseline.

I claim,

A composition resulting from a mixture of 4 oz. paraffin oil,  $1\frac{1}{2}$  oz. turpentine, 3 oz. alcohol,  $\frac{1}{8}$  oz. acetic acid,  $\frac{1}{2}$  oz. ammonia,  $1\frac{1}{2}$  oz. Putz pomade, 1 oz. ivory soap and 2 oz. water.

ROY A. ALEXANDER.